

Oct. 9, 1973

KEISUKE SKIBA ET AL  
SPECTRALLY SENSITIZED SILVER HALIDE  
PHOTOGRAPHIC EMULSION  
Filed Sept. 24, 1971

3,764,340

FIG1



FIG2



FIG3



FIG4



3,764,340

## SPECTRALLY SENSITIZED SILVER HALIDE PHOTOGRAPHIC EMULSION

Keisuke Shiba, Haruo Takei, Akira Sato, and Tadashi Ikeda, Kanagawa, Japan, assignors to Fuji Photo Film Co., Ltd., Kanagawa, Japan

Filed Sept. 24, 1971, Ser. No. 183,592

Claims priority, application Japan, Sept. 24, 1970,  
45/83,656

Int. Cl. G03c 1/14

U.S. Cl. 96—124

6 Claims

### ABSTRACT OF THE DISCLOSURE

A spectrally sensitized silver halide photographic emulsion, and more particularly a silver halide photographic emulsion supersensitized by the combined use of at least two sensitizing dyes resulting in a high red sensitivity.

### FIELD OF THE INVENTION

This invention relates to a spectrally sensitized silver halide photographic emulsion, and more particularly to a silver halide photographic emulsion which is supersensitized by the combined use of at least two sensitizing dyes resulting in a high red sensitivity.

### BACKGROUND OF THE INVENTION

#### (1) Prior art

Photographic light-sensitive materials which are used conventionally are required to have spectral sensitivity distribution corresponding to the photographing purpose. However, for the manufacture of the sensitive material, it is difficult to develop a combination of sensitizing dyes which are in the supersensitization relation to each other and which has a small inherent desensitization, i.e. a low desensitization in the wavelength region inherent to silver halide grains.

#### (2) Objects of the invention

An object of this invention is to provide a silver halide photographic emulsion having a high red sensitivity within the spectrally sensitized wavelength region of 620–685 nm. and a small inherent desensitization by the combined use of two different types of sensitizing dyes. In particular, it aims at the improved red sensitivity of black-and-white sensitive material having a sensitive maximum in the vicinity of 630 nm. and the improved spectral sensitivity of black-and-white sensitive material having a sensitive maximum in a longer wavelength region, i.e. in the region of 640–680 nm.

Other objects of this invention will be apparent to those skilled in the art as the description of this invention proceeds.

### DESCRIPTION OF THE INVENTION

This invention is the combined use of sensitizing dyes of the following general Formulas I and II in a silver halide photographic emulsion:



wherein R<sub>1</sub> represents a lower alkyl group, e.g., methyl, ethyl, propyl, etc., alkenyl, e.g., vinyl, methyl, etc.; R<sub>2</sub> represents a sulfoalkyl group, e.g.,  $\gamma$ -sulfopropyl,  $\gamma$ -sulfobutyl,  $\delta$ -sulfobutyl, etc.; A<sub>1</sub> represents a lower alkyl group, e.g., methyl, ethyl, etc., or an aryl group, e.g., phenyl, p-methoxyphenyl; Z<sub>1</sub> represents nonmetallic atoms required to complete a benzothiazole, benzoselenazole or  $\beta$ -naphthothiazole nucleus, which may be substituted by a halogen atom, e.g., chlorine, bromine atom, etc., a lower alkyl group, e.g., methyl, ethyl, etc., an alkoxy group, e.g., methoxy, etc., an aryl group, e.g., phenyl; Z<sub>2</sub> represents a sulfur or a selenium atom, B represents a phenyl group which may be a substituted phenyl group, or

quired to complete a benzothiazole, benzoselenazole or  $\beta$ -naphthothiazole nucleus, which may be substituted by a halogen atom, e.g., chlorine, bromine atom, etc., a lower alkyl group, e.g., methyl, ethyl, etc., an alkoxy group, e.g., methoxy, etc., an aryl group, e.g., phenyl; Z<sub>2</sub> represents a sulfur or a selenium atom, B represents a phenyl group which may be a substituted phenyl group, or



wherein P and Q represent hydrogen atoms or lower alkyl groups or an atomic group capable of being connected to each other to form a heterocyclic ring; X<sub>1</sub><sup>-</sup> represents an anion, e.g., chloride, bromide, iodide, p-toluenesulfonate ion, etc., which are used generally in the field of sensitizing dyes, n is 0 or 1 and n=0 for intermolecular salt;

wherein R<sub>3</sub> and R<sub>4</sub> each represents a lower alkyl group, e.g., methyl, ethyl, propyl,  $\gamma$ -sulfopropyl,  $\gamma$ -sulfobutyl,  $\delta$ -sulfobutyl,  $\delta$ -carboxybutyl, etc.; A<sub>2</sub> represents a lower alkyl group, e.g., methyl, ethyl, etc., or an aryl group, e.g., phenyl; Z<sub>3</sub> and Z<sub>4</sub> each represents nonmetallic atoms required to complete a benzothiazole, benzoselenazole or  $\beta$ -naphthothiazole nucleus, which may be substituted by a halogen atom, e.g., chlorine, bromine atom, etc., a lower alkyl group, e.g., methyl, ethyl, etc., an alkoxy group, e.g., methoxy, ethoxy, etc., a hydroxyl group, carboxyl group, alkoxy carbonyl group, e.g., methoxycarbonyl, ethoxycarbonyl, etc., and phenyl group, etc.; X<sub>2</sub><sup>-</sup> represents an anion, e.g., chloride, bromide, iodide, p-toluenesulfonate ion, etc., which are used generally in the field of sensitizing dyes; m is 0 or 1 and m=0 for the intermolecular salt.

The cyanine dyes of the general Formula I have a sensitized maximum peak in the range of 620–650 nm. and, compared with the sensitizing dyes of the general Formula II, a very small red sensitivity. Many cyanine dyes of the general Formula II have a sharp J-band and a high red sensitivity. It has been found that the combined use of said sensitizing dyes (I) and (II) having such features improves the red sensitivity of said sensitizing dye of (II), resulting in a silver halide photographic emulsion having a very small inherent desensitization. Above all, the combination of said sensitizing dye of (I) and mesomethylthiacarbocyanine among said sensitizing dye (II) is suitable to a black-and-white sensitive material having a sensitized maximum peak in the vicinity of 630 nm. and shows such effect that has not been found in the previous art, said effect extending gradually the spectral sensitization region to the longer wavelength without a large shift of sensitive maximum peak. The combination use of a sensitizing dye of the general Formula I and a symmetrical  $\beta$ -naphthothiacarbocyanine of the general Formula II has a peculiar effect: that is, the sensitized maximum peak may be selected voluntarily in the region of 620–680 nm. and the spectral sensitivity can be highly increased to maintain the red sensitivity at a high level. Said effect is not affected by using at the same time another sensitizer for improving the green sensitivity (for example, 2,2'-cyanine, thia-2'-cyanine, etc.) or sensitizers having other spectral sensitization region.

The FIGS. 1–4 show the sensitivities of the dyes described herein when compared with various control samples. A fuller understanding of the drawings can be had by referring to Table 2 and the specific examples reported therein.

The embodiment of sensitizing dyes used in this invention are mentioned as follows, but said sensitizing dyes used in this invention are not restricted to these examples.



Dye D



Dye E



Dye F



Dye G



Dye H



Dye I



Dye J



Dye K



Dye L



The sensitizing dyes of the general Formulas I and II, which are used in this invention, can be synthesized by a known method. For example, by reference to U.S. Pat. No. 2,503,776 and German Pat. Nos. 929,080 and 1,072,765, those skilled in the art can synthesize them readily.

Typical syntheses of new sensitizing dyes of the general Formula I are described as follows:

Synthesis (i): Dye (I)-1

10 3.0 g. of 5-chloro-3-propyl-2-thiopropionylmethylenebenzothiazoline and 4.5 ml. of methyl-p-toluenesulfonate were heated at 110° C. for one hour and, after cooling, treated with ethyl ether to remove the unreacted material. 3.6 g. of anhydro-5-N,N-dimethylcarbamoyl-3-( $\gamma$ -sulfopropyl)-2-methylbenzothiazolium hydroxide, 400 ml. of ethanol and 5 ml. of triethylamine were added and heated for 3 hours under reflux and the solvent was then removed. The remainder was treated with ether and then with a mixed solvent of ethanol/acetone thoroughly to yield coarse crystals, which were recrystallized from a mixed solvent of isopropanol/ethanol to yield 1.7 g. of dye. M.P. 270.5° C.;

$\lambda_{\text{max}}^{\text{MeOH}}$  557 nm.

25 Analysis for  $\text{C}_{28}\text{H}_{32}\text{N}_3\text{S}_3\text{O}_4\text{Cl}$  (M.W.=606.2).—Calculated (percent): C, 55.85; H, 5.36; N, 6.97. Found (percent): C, 55.67; H, 5.31; N, 6.97.

Synthesis (ii): Dye (I)-2

30 1 g. of 5-chloro-3-allyl-2-thiopropionylmethylenebenzothiazoline and 1.5 ml. of methyl-p-toluenesulfonate were heated at 115° C. for 1.5 hours and the unreacted solid was then washed with ether, 1 g. of anhydro-5-benzoyl-3-( $\gamma$ -sulfopropyl)-2-methylthiazolium hydroxide, 200 ml. of ethanol and 1.5 ml. of triethylamine were then added and heated for 2.5 hours under reflux. The solvent was removed and the remainder was treated with ether and then with acetone thoroughly to yield coarse crystals, which were recrystallized from a mixed solvent of ethanol/methanol to yield 650 mg. of dye. M.P. 286° C.;

$\lambda_{\text{max}}^{\text{MeOH}}$  558 nm.

35 Analysis for  $\text{C}_{32}\text{H}_{29}\text{N}_2\text{S}_3\text{O}_4\text{Cl}$  (M.W.=637.2).—Calculated (percent): C, 60.25; H, 4.59; N, 4.39. Found (percent): C, 59.83; H, 4.69; N, 4.29.

Synthesis (iii): Dye (I)-7

40 1 g. of 5-chloro-3-ethyl-2-thiopropionylmethylenebenzothiazoline and 1.5 ml. of methyl-p-toluenesulfonate were reacted at 115° C. for 2 hours with heating and the reaction mixture was then washed with ether. 1 g. of anhydro-5-benzoyl-3-( $\gamma$ -sulfopropyl)-2-methylbenzothiazolium hydroxide, 200 ml. of ethanol and 2 ml. of triethylamine were then added and heated for 3 hours under reflux. After completion of the reaction, the solvent was removed and the remainder was washed with ether and then with a mixed solvent of ethanol/acetone to yield coarse crystals, which were recrystallized from a mixed solvent of ethanol/methanol/chloroform to yield 800 mg. of dye crystal. M.P. above 308° C.;

$\lambda_{\text{max}}^{\text{MeOH}}$  553 nm.

45 Analysis for  $\text{C}_{36}\text{H}_{31}\text{N}_2\text{S}_3\text{O}_5\text{Cl}$  (M.W.=703.3).—Calculated (percent): C, 61.48; H, 4.44; N, 3.98. Found (percent): C, 61.49; H, 4.55; N, 3.85.

Synthesis (iv): Dye (I)-10

50 1 g. of 5-methyl-3-ethyl-2-thiopropionylmethylenebenzothiazoline and 1.5 ml. of methyl-p-toluenesulfonate were reacted at 110° C. for 2 hours with heating and then washed with ether. To the remainder was added 1.2 g. of anhydro-5-ethylcarbamoyl-3-( $\gamma$ -sulfopropyl)-2-methylbenzothiazolium hydroxide, 140 ml. of ethanol and 4 ml. of triethylamine and the admixture was heated for 3.5 hours under reflux. The solvent was then removed and the remainder washed with ether and then with ethanol/ether

to yield coarse crystals, which were washed with acetone and recrystallized twice from a mixed solvent of ethanol/isopropanol to yield 550 mg. of dye. M.P. above 300° C.;

$\lambda_{\text{max}}^{\text{MeOH}}$  555 nm.

Analysis for  $\text{C}_{23}\text{H}_{33}\text{N}_3\text{S}_3\text{O}_4$  (M.W.=571.8).—Calculated (percent): C, 58.75; H, 5.81; N, 7.34. Found (percent): C, 58.52; H, 5.80; N, 6.95.

Synthesis (v): Dye (I)-14

0.85 g. of 5-chloro-3-ethyl-2-thiopropionylmethylenbenzoselenazoline and 1.5 ml. of methyl-p-toluene sulfonate were reacted at 110° C. for 1.5 hours on an oil bath. After cooling, the reacted solid was washed with ether, 1.25 g. of anhydro-5-morpholinocarbonyl-3-( $\gamma$ -sulfopropyl)-2-methylbenzothiazolium hydroxide were added to the solid and reacted for one hour on an oil bath with heating under reflux in 130 ml. of ethanol and 3 ml. of triethylamine. Thereafter, the solvent was distilled off and the remainder was treated first with ethanol/ether and then with acetone to yield coarse crystals, which were recrystallized from a mixed solvent of ethanol/isopropanol to yield 170 mg. of dye. M.P. 261° C.;

$\lambda_{\text{max}}^{\text{MeOH}}$  563 nm.

Analysis for  $\text{C}_{23}\text{H}_{32}\text{N}_3\text{S}_2\text{SeO}_5\text{Cl}$  (M.W.=679.1).—Calculated (percent): C, 51.27; H, 4.74; N, 6.18. Found (percent): C, 51.30; H, 4.78; N, 6.09.

Other sensitizing dyes according to this invention can be similarly synthesized.

The spectral sensitization process according to this invention is effective for the spectral sensitization of gelatin silver halide photographic emulsion. It can also sensitize sufficiently an emulsion containing hydrophilic colloid other than gelatin, e.g., agar colloidion, water-soluble cellulose derivatives, polyvinyl alcohol or other synthetic or natural hydrophilic resins. For the photographic emulsion used in this invention, a mixed silver halide emulsion such as silver iodobromide, chloroiodobromide, etc., are suitable.

For the preparation of spectrally sensitized photographic emulsion according to this invention, it is possible to add said sensitizing dye of (I) and (II) to a photographic emulsion in a common manner. In practice, it is convenient to add the dyes as a solution in a suitable solvent such as methanol, ethanol, etc., to the emulsion.

The sensitizing dyes (I) and (II) to be contained in the emulsion are used in an amount of  $10^{-6}$  to  $10^{-3}$  mol/mol of silver halide respectively and the molar ratio of both dyes may be varied within a wide range of from 9:1 to

1:9 corresponding to the effect desired. The photographic emulsion according to this invention can be applied further with the hyper- and other super-sensitization. In the preparation of the photographic emulsion according to this invention, additives which are generally used, for example, chemical sensitizer, stabilizer, toner, hardener, surface active agent, antifoggant, plasticizer, development accelerator, color developer and fluorescent brightening agent can be contained in the emulsion in a common manner.

The photographic emulsion according to this invention can be coated on a suitable base, for example, glass, films of cellulose derivatives, films of synthetic resins, baryta paper or resin-coated paper in a common manner.

Examples are described as follows:

20 Single sensitizing dye of (I) and (II) used in this invention each was added to a silver iodobromide emulsion (AgI:AgBr—7:93 in mol percent) to prepare silver halide photographic emulsions. On the other hand, silver halide photographic emulsions containing the combination of said sensitizing dyes of (I) and (II) used in this invention were prepared. These emulsions were coated respectively on a cellulose triacetate film base, dried, then exposed through a yellow filter (a filter transmitting rays of longer wavelength than 580 nm.) and a blue filter (a filter transmitting rays of 400-490 nm. and having a maximum transmission at 450 nm.) to a daylight of 64 luxes (corresponding to 5,400° K.) and developed. As the liquid developer, one having the composition shown in Table 1 was used.

TABLE 1

|                    |       | G.  |
|--------------------|-------|-----|
| Metol              | ----- | 2   |
| Sodium sulfite     | ----- | 100 |
| Hydroquinone       | ----- | 5   |
| 40 Borax           | ----- | 2   |
| Water to make 1 l. |       |     |

The relative yellow sensitivity, relative red sensitivity and inherent desensitization to the original emulsion in the single addition of said sensitizing dyes (I) and (II) as well as in the combined use of said sensitizing dyes (I) and (II) are shown in Table 2.

TABLE 2

| Experiment No. | Example No. | Dye No. | Amount of sensitizing dye added <sup>1</sup> | Dye No. | Amount of sensitizing dye added <sup>1</sup> | Emulsion | Sensitized maximum (nm.) | Relative yellow sensitivity | Relative red sensitivity | Inherent sensitivity | Refer to— |            |
|----------------|-------------|---------|----------------------------------------------|---------|----------------------------------------------|----------|--------------------------|-----------------------------|--------------------------|----------------------|-----------|------------|
| 1              | 1           | 1       | J                                            | 0.5     | AgBr/I                                       | 635      | 62                       | 77                          | 96                       | FIG. 1 (1)           |           |            |
|                |             |         | J                                            | 1       | AgBr/I                                       | 636      | 105                      | 150                         | 96                       | FIG. 1 (2)           |           |            |
|                |             |         | J                                            | 2       | AgBr/I                                       | 636      | 115                      | 160                         | 90                       | FIG. 1 (3)           |           |            |
|                |             |         | J                                            | 4       | AgBr/I                                       | 636      | 135                      | 185                         | 60                       |                      |           |            |
|                |             |         | J                                            | 6       | AgBr/I                                       | 620      | 68                       | 32                          | 100                      |                      |           |            |
|                |             |         | J                                            | 8       | AgBr/I                                       | 628      | 76                       | 40                          | 100                      | FIG. 4 (10)          |           |            |
| 2              | 2           | 1       | 1                                            | 4       | J                                            | 0.5      | AgBr/I                   | 630                         | 250                      | 200                  | 96        |            |
|                |             |         | 1                                            | 4       | J                                            | 1        | AgBr/I                   | 685                         | 280                      | 250                  | 90        |            |
|                |             |         | 1                                            | 4       | J                                            | 2        | AgBr/I                   | 685                         | 280                      | 260                  | 90        |            |
|                |             |         | 6                                            | 2       | AgBr/I                                       | 635      | 64                       | 40                          | 100                      |                      |           |            |
|                |             |         | 6                                            | 4       | AgBr/I                                       | 638      | 94                       | 44                          | 88                       |                      |           |            |
|                |             |         | 6                                            | 8       | AgBr/I                                       | 638      | 96                       | 44                          | 62                       |                      |           |            |
| 3-a            | 3-a         | 2       | 6                                            | 4       | J                                            | 0.5      | AgBr/I                   | 620-650                     | 225                      | 210                  | 94        |            |
|                |             |         | 6                                            | 4       | J                                            | 1        | AgBr/I                   | 620-660                     | 270                      | 260                  | 90        |            |
|                |             |         | 12                                           | 2       | AgBr/I                                       | 630      | 85                       | 57                          | 85                       |                      |           |            |
|                |             |         | 12                                           | 4       | AgBr/I                                       | 630      | 82                       | 57                          | 83                       | FIG. 2 (4)           |           |            |
|                |             |         | 12                                           | 8       | AgBr/I                                       | 630      | 80                       | 54                          | 64                       |                      |           |            |
|                |             |         | 12                                           | 4       | J                                            | 0.5      | AgBr/I                   | 620-640                     | 240                      | 225                  | 90        | FIG. 2 (5) |
| 3-b            | 3-b         | 3       | 12                                           | 4       | J                                            | 1        | AgBr/I                   | 630                         | 280                      | 280                  | 90        | FIG. 2 (6) |
|                |             |         | 12                                           | 4       | J                                            | 2        | AgBr/I                   | 630                         | 300                      | 310                  | 85        | FIG. 2 (7) |
|                |             |         | 12                                           | 2       | J                                            | 0.5      | AgBr/I                   | 620-660                     | 230                      | 280                  | 94        |            |
|                |             |         | 12                                           | 2       | J                                            | 1        | AgBr/I                   | 620-670                     | 300                      | 290                  | 90        |            |
|                |             |         | 12                                           | 2       | J                                            | 2        | AgBr/I                   | 630                         | 330                      | 345                  | 88        |            |
|                |             |         | 12                                           | 2       | J                                            | 16       | 2 {AgBr/I                | 678                         | 350                      | 360                  | 90        |            |

TABLE 2.—Continued

| Experiment No. | Example No. | Dye No. | Amount of sensitizing dye added <sup>1</sup> | Dye No. | Amount of sensitizing dye added <sup>1</sup> | Emulsion | Sensitized maximum (nm.) | Relative yellow sensitivity | Relative red sensitivity | Inherent sensitivity | Refer to—   |
|----------------|-------------|---------|----------------------------------------------|---------|----------------------------------------------|----------|--------------------------|-----------------------------|--------------------------|----------------------|-------------|
| 4              |             | 10      | 2                                            |         |                                              | AgBr/I   | 620                      | 35                          | 32                       | 94                   |             |
|                |             | 10      | 4                                            |         |                                              | AgBr/I   | 625                      | 66                          | 45                       | 89                   |             |
|                |             | 10      | 8                                            |         |                                              | AgBr/I   | 630                      | 66                          | 50                       | 75                   |             |
| 5              | 5           | 10      | 4                                            | J       | 1                                            | AgBr/I   | 650                      | 100                         | 93                       | 76                   |             |
|                |             | 10      | 4                                            | J       | 2                                            | AgBr/I   | 655                      | 158                         | 153                      | 76                   |             |
|                |             | 10      | 4                                            | J       | 4                                            | AgBr/I   | 660                      | 142                         | 142                      | 60                   |             |
|                |             | 4       | 2                                            |         |                                              | AgBr/I   | 638                      | 32                          | 8                        | 94                   |             |
| 6              | 6           | 4       | 4                                            |         |                                              | AgBr/I   | 638                      | 40                          | 18                       | 85                   |             |
|                |             | 4       | 8                                            |         |                                              | AgBr/I   | 638                      | 45                          | 27                       | 85                   |             |
|                |             | 4       |                                              | G       | 1                                            | AgBr/I   | 650                      | 58                          | 43                       | 98                   |             |
|                | 7           | 4       |                                              | G       | 2                                            | AgBr/I   | 650                      | 90                          | 90                       | 98                   |             |
|                |             | 4       |                                              | G       | 4                                            | AgBr/I   | 650                      | 120                         | 110                      | 98                   |             |
|                |             | 4       |                                              | G       | 8                                            | AgBr/I   | 650                      | 120                         | 105                      | 85                   |             |
|                | 4           | 4       | G                                            | 1       | AgBr/I                                       | 646      | 135                      | 140                         | 98                       |                      |             |
|                | 4           | 4       | G                                            | 2       | AgBr/I                                       | 646      | 140                      | 140                         | 98                       |                      |             |
| 7              | 7           | 3       | 2                                            |         |                                              | AgBr/I   | 628                      | 74                          | 37                       | 90                   |             |
|                |             | 3       | 4                                            |         |                                              | AgBr/I   | 628                      | 82                          | 40                       | 90                   |             |
|                |             | 3       | 8                                            |         |                                              | AgBr/I   | 630                      | 86                          | 44                       | 85                   |             |
|                |             | 3       |                                              | H       | 2                                            | AgBr/I   | 652                      | 85                          | 75                       | 98                   |             |
| 8              | 8           | 3       | 2                                            | H       | 4                                            | AgBr/I   | 650                      | 130                         | 115                      | 95                   |             |
|                |             | 3       | 4                                            | H       | 4                                            | AgBr/I   | 648                      | 160                         | 130                      | 95                   |             |
|                |             | 8       | 1                                            |         | AgBr/I                                       | 646      | 27                       | 14                          | 95                       |                      |             |
|                |             | 8       | 2                                            |         | AgBr/I                                       | 646      | 30                       | 18                          | 95                       |                      |             |
|                |             | 8       | 4                                            |         | AgBr/I                                       | 646      | 33                       | 20                          | 88                       |                      |             |
| 9              | 9           | 8       | 1                                            | H       | 4                                            | AgBr/I   | 656                      | 120                         | 125                      | 95                   |             |
|                |             | 8       | 2                                            | H       | 4                                            | AgBr/I   | 656                      | 125                         | 125                      | 95                   |             |
|                |             | 1       | 4                                            | I       | 1                                            | AgBr/I   | 635                      | 35                          | 35                       | 90                   |             |
|                |             | 1       | 4                                            | I       | 2                                            | AgBr/I   | 685                      | 70                          | 70                       | 85                   |             |
| 10-a           | 10          | 1       | 4                                            | I       | 1                                            | AgBr/I   | 620                      | 315                         | 315                      | 100                  |             |
|                |             | 1       | 4                                            | I       | 2                                            | AgBr/I   | 620-685                  | 223                         | 224                      | 100                  | FIG. 4 (11) |
|                |             | 1       | 4                                            | I       | 4                                            | AgBr/I   | 620-685                  | 178                         | 165                      | 89                   |             |
|                |             | 7       | 2                                            |         |                                              | AgBr/I   | 610                      | 47                          | 15                       | 80                   |             |
| 10-b           | 11          | 7       | 4                                            |         |                                              | AgBr/I   | 640                      | 47                          | 20                       | 74                   |             |
|                |             | 7       | 8                                            |         |                                              | AgBr/I   | 640                      | 43                          | 22                       | 73                   |             |
|                |             | 7       | 4                                            | J       | 0.5                                          | AgBr/I   | 670-680                  | 111                         | 155                      | 98                   |             |
|                |             | 7       | 4                                            | J       | 1                                            | AgBr/I   | 680                      | 160                         | 193                      | 90                   |             |
| 11             | 12          | 2       | 1                                            | A       | 4                                            | AgBr/I   | 632                      | 30                          | 18                       | 98                   |             |
|                |             | 2       | 2                                            |         |                                              | AgBr/I   | 632                      | 48                          | 26                       | 94                   |             |
|                |             | 2       | 4                                            |         |                                              | AgBr/I   | 632                      | 62                          | 40                       | 85                   | FIG. 3 (12) |
|                |             | 2       | 8                                            |         |                                              | AgBr/I   | 635                      | 66                          | 47                       | 76                   |             |
| 12             | 13          | A       | 2                                            |         | 2                                            | AgBr/I   | 600                      | 140                         | 38                       | 94                   |             |
|                |             | A       | 4                                            |         | 4                                            | AgBr/I   | 630                      | 230                         | 90                       | 92                   | FIG. 3 (8)  |
|                |             | A       | 8                                            |         | 8                                            | AgBr/I   | 632                      | 260                         | 115                      | 80                   |             |
|                |             | 2       | 1                                            | A       | 4                                            | AgBr/I   | 632                      | 320                         | 130                      | 100                  | FIG. 3 (9)  |
| 13             | 14          | 2       | 16                                           | A       | 4                                            | AgBr/I   | 630                      | 355                         | 130                      | 100                  |             |
|                |             | 5       | 2                                            |         |                                              | AgBr/I   | 638                      | 22                          | 6                        | 96                   |             |
|                |             | 5       | 4                                            |         |                                              | AgBr/I   | 638                      | 26                          | 14                       | 85                   |             |
|                |             | 5       | 8                                            |         |                                              | AgBr/I   | 638                      | 30                          | 20                       | 85                   |             |
| 14             | 15          | B       | 2                                            |         | 2                                            | AgBr/I   | 600                      | 95                          | 23                       | 92                   |             |
|                |             | B       | 4                                            |         | 4                                            | AgBr/I   | 630                      | 130                         | 55                       | 90                   |             |
|                |             | 5       | 2                                            | B       | 4                                            | AgBr/I   | 636                      | 180                         | 85                       | 90                   |             |
|                |             | 5       | 2                                            | B       | 4                                            | AgBr/I   | 638                      | 200                         | 100                      | 90                   |             |
| 15             | 16          | D       | 4                                            |         |                                              | AgBr/I   | 622                      | 180                         | 40                       | 90                   |             |
|                |             | 12      | 1                                            | D       | 4                                            | AgBr/I   | 632                      | 180                         | 65                       | 90                   |             |
|                |             | 12      | 2                                            | D       | 4                                            | AgBr/I   | 634                      | 180                         | 78                       | 90                   |             |
|                |             | F       | 1                                            |         | AgBr/I                                       | 640-645  | 110                      | 48                          | 85                       |                      |             |
| 16             | 17          | F       | 2                                            |         | 2                                            | AgBr/I   | 655-658                  | 150                         | 78                       | 58                   |             |
|                |             | 15      | 2                                            |         |                                              | AgBr/I   | 630                      | 51                          | 40                       | 94                   |             |
|                |             | 15      | 4                                            |         |                                              | AgBr/I   | 630                      | 51                          | 30                       | 80                   |             |
|                |             | 15      | 8                                            |         |                                              | AgBr/I   | 632                      | 57                          | 33                       | 78                   |             |
| 17             | 18          | 15      | 4                                            | F       | 1                                            | AgBr/I   | 640                      | 200                         | 120                      | 90                   |             |
|                |             | 15      | 4                                            | F       | 2                                            | AgBr/I   | 645                      | 230                         | 165                      | 90                   |             |
|                |             | 13      | 2                                            |         |                                              | AgBr/I   | 620                      | 63                          | 45                       | 93                   |             |
|                |             | 13      | 4                                            |         |                                              | AgBr/I   | 620                      | 76                          | 45                       | 93                   |             |
| 18             | 19          | 13      | 8                                            |         |                                              | AgBr/I   | 620                      | 85                          | 50                       | 89                   |             |
|                |             | 13      | 4                                            | J       | 1                                            | AgBr/I   | 620                      | 132                         | 105                      | 71                   |             |
|                |             | 13      | 4                                            | J       | 2                                            | AgBr/I   | 620                      | 142                         | 135                      | 69                   |             |
|                |             | 13      | 4                                            | J       | 4                                            | AgBr/I   | 620-680                  | 142                         | 152                      | 66                   |             |
| 19             | 20          | 13      | 2                                            | H       | 4                                            | AgBr/I   | 645                      | 100                         | 100                      | 78                   |             |
|                |             | 13      | 4                                            | H       | 4                                            | AgBr/I   | 645                      | 138                         | 100                      | 78                   |             |
|                |             | 13      | 8                                            | H       | 4                                            | AgBr/I   | 635                      | 158                         | 120                      | 78                   |             |
|                |             | 11      | 2                                            |         |                                              | AgBr/I   | 605                      | 50                          | 22                       | 100                  |             |
| 20             | 21          | 11      | 4                                            |         |                                              | AgBr/I   | 615                      | 76                          | 76                       | 100                  |             |
|                |             | 11      | 4                                            |         |                                              | AgBr/I   | 620                      | 100                         | 100                      | 89                   |             |
|                |             | 11      | 8                                            |         |                                              | AgBr/I   | 620                      | 100                         | 100                      | 89                   |             |
|                |             | 11      | 4                                            | J       | 1                                            | AgBr/I   | 620                      | 200                         | 132                      | 100                  |             |
| 21             | 22          | 11      | 4                                            | J       | 2                                            | AgBr/I   | 620-680                  | 200                         | 152                      | 93                   |             |
|                |             | 11      | 4                                            | J       | 4                                            | AgBr/I   | 680                      | 200                         | 180                      | 71                   |             |
|                |             | 11      | 4                                            | J       | 4                                            | AgBr/I   | 620                      | 200                         | 180                      | 71                   |             |

TABLE 2.—Continued

| Experiment No. | Example No. | Dye No. | Amount of sensitizing dye added <sup>1</sup> | Dye No. | Amount of sensitizing dye added <sup>1</sup> | Emulsion | Sensitized maximum (nm.) | Relative yellow sensitivity | Relative red sensitivity | Inherent sensitivity | Refer to— |
|----------------|-------------|---------|----------------------------------------------|---------|----------------------------------------------|----------|--------------------------|-----------------------------|--------------------------|----------------------|-----------|
| 17             |             |         | K                                            |         | 2 AgBr/I                                     | 650      | 107                      | 100                         | 96                       |                      |           |
|                |             |         | K                                            |         | 4 AgBr/I                                     | 650      | 115                      | 115                         | 89                       |                      |           |
|                |             |         | K                                            |         | 8 AgBr/I                                     | 650      | 142                      | 142                         | 83                       |                      |           |
| 18             | 19          | 11      | 1                                            | K       | 4 AgBr/I                                     | 650      | 166                      | 150                         | 100                      |                      |           |
|                |             | 11      | 2                                            | K       | 4 AgBr/I                                     | 640      | 200                      | 200                         | 100                      |                      |           |
|                |             | 11      | 4                                            | K       | 4 AgBr/I                                     | 640      | 214                      | 214                         | 96                       |                      |           |
| 18             | 20          | 14      | 2                                            |         | AgBr/I                                       | 610      | 35                       | 22                          | 63                       |                      |           |
|                |             | 14      | 4                                            |         | AgBr/I                                       | 625      | 45                       | 25                          | 55                       |                      |           |
|                |             | 14      | 4                                            | J       | 1 AgBr/I                                     | 520      | 110                      | 110                         | 66                       |                      |           |
| 20             | 21          | 14      | 4                                            | J       | 2 AgBr/I                                     | 620      | 142                      | 142                         | 66                       |                      |           |
|                |             | 14      | 4                                            | J       | 4 AgBr/I                                     | 620-680  | 141                      | 142                         | 60                       |                      |           |
|                |             |         |                                              | C       | 6 AgBr/I                                     | 632      | 150                      | 76                          | 78                       |                      |           |
| 21             | 21          | 12      | 1                                            | C       | 6 AgBr/I                                     | 632      | 160                      | 85                          | 78                       |                      |           |
|                |             | 12      | 2                                            | C       | 6 AgBr/I                                     | 632      | 165                      | 85                          | 75                       |                      |           |
| 20             | 22          |         |                                              | E       | 6 AgBr/I                                     | 646      | 140                      | 125                         | 45                       |                      |           |
|                |             | 15      | 2                                            | E       | 6 AgBr/I                                     | 646      | 152                      | 130                         | 66                       |                      |           |
|                |             | 15      | 1                                            | B       | 4 AgBr/I                                     | 632      | 146                      | 110                         | 87                       |                      |           |
| 22             | 23          | 15      | 2                                            | B       | 4 AgBr/I                                     | 632      | 144                      | 110                         | 87                       |                      |           |
|                |             | 9       | 2                                            |         | AgBr/I                                       | 644      | 44                       | 48                          | 98                       |                      |           |
|                |             | 9       | 4                                            |         | AgBr/I                                       | 644      | 73                       | 60                          | 86                       |                      |           |
| 22             | 24          | 9       | 8                                            |         | AgBr/I                                       | 646      | 78                       | 64                          | 84                       |                      |           |
|                |             |         |                                              | L       | 1 AgBr/I                                     | 634      | 66                       | 38                          | 95                       |                      |           |
|                |             |         |                                              | L       | 2 AgBr/I                                     | 636      | 82                       | 54                          | 92                       |                      |           |
| 23             | 25          |         |                                              | L       | 4 AgBr/I                                     | 640-645  | 85                       | 62                          | 88                       |                      |           |
|                |             | 9       | 4                                            | L       | 2 AgBr/I                                     | 646      | 100                      | 76                          | 78                       |                      |           |
|                |             | 8       | 1                                            |         | AgBr/I                                       | 646      | 25                       | 13                          | 94                       |                      |           |
| 23             | 25          | 8       | 2                                            |         | AgBr/I                                       | 646      | 27                       | 17                          | 94                       |                      |           |
|                |             | 8       | 4                                            |         | AgBr/I                                       | 646      | 30                       | 19                          | 85                       |                      |           |
|                |             | 8       | 1                                            | H       | 4 AgBr/I                                     | 656      | 110                      | 110                         | 94                       |                      |           |
|                |             | 8       | 2                                            | H       | 4 AgBr/I                                     | 656      | 112                      | 110                         | 92                       |                      |           |

<sup>1</sup> 10<sup>-5</sup> mol/kg. emulsion.

The yellow and red sensitivity are each shown as the relative sensitivity to the sensitivity 100 of said sensitizing dye H which is exposed in an amount of 4×10<sup>-5</sup> mol/kg. emulsion through the yellow and red filter as mentioned above and the inherent sensitivity is shown as the relative sensitivity to the sensitivity 100 of original emulsion which is exposed through the blue filter.

As can be seen from Table 2, the combined use of said sensitizing dyes (I) and (II) provides a much higher spectral sensitization than in the single use of each sensitizing dye.

As shown in Table 2 and Examples 3, 4, 11 and 12, the effect of the combination of said sensitizing dyes (I) and (II) is not injured by the further addition of known green sensitizing dye thereto, i.e. the combined use of green sensitizing dye 16 or 17 with the combination of said sensitizing dyes (I) and (II).

The green sensitizing dyes which may be used in combination with said sensitizing dye of (I) and (II) used in this invention are those having the following chemical structures, but they are not restricted only to these sensitizing dyes.

## GREEN SENSITIZING DYE

(16)



(17)



What is claimed is:

1. A silver halide photographic emulsion containing the supersensitizing combination of at least one of sensitizing

dyes of the general Formula I and at least one of sensitizing dyes of the general Formula II:



wherein  $R_1$  represents a lower alkyl or alkenyl group,  $R_2$  represents a sulfoalkyl group,  $A_1$  represents a lower alkyl, or aryl group,  $Z_1$  represents a nonmetallic atom required to complete a benzothiazole, benzoselenazole or  $\beta$ -naphthothiazole nucleus,  $Z_2$  represents a sulfur or selenium atom,  $B$  represents a phenyl, or

group, wherein  $P$  and  $Q$  each represents a hydrogen atom or a lower alkyl group or an atomic group capable of being connected to form a morpholine ring,  $X_1^-$  represents an anion,  $n$  is 0 or 1,  $n$  being 0 for the intermolecular salt;



wherein  $R_3$  and  $R_4$  each represents a lower alkyl group,  $A_2$  represents a lower alkyl or aryl group,  $Z_3$  and  $Z_4$  each represents a nonmetallic atom required to complete a benzothiazole, benzoselenazole or  $\beta$ -naphthothiazole nucleus,  $X_2^-$  represents an anion,  $m$  is 0 or 1,  $m$  being 0 for the intermolecular salt.

2. A silver halide photographic emulsion as claimed in claim 1 wherein the sensitizing dye of the general Formula II is a mesomethylthiacyarbocyanine.

3. A silver halide photographic emulsion as claimed in claim 1 wherein the sensitizing dye of the general Formula II is a symmetrical  $\beta$ -naphthothiacyarbocyanine.

13. 4. A silver halide photographic emulsion as claimed in claim 1, wherein said emulsion further contains a green sensitizing dye selected from the group consisting of 2,2'-cyanine and thia-2'-cyanine.

**5.** A silver halide photographic emulsion as claimed in claim 1 wherein the sensitizing dye of the general Formula I is a member selected from the group consisting of:



15



16



30 6. A photographic light-sensitive material comprising a layer containing the photographic emulsion as claimed in claim 1.

References Cited

UNITED STATES PATENTS

35 2,521,705 9/1950 Firestone ----- 96—137  
3,468,661 9/1969 Libeer et al. ----- 96—137  
3,681,080 8/1972 Nakazawa et al. ----- 96—124

40 I. TRAVIS BROWN, Primary Examiner

U.S. Cl. X.R.

96—137